

July 28, 1959

H. C. L. DUNKER

2,896,949

TENNIS BALLS

Filed March 15, 1954



FIG. 1



FIG. 2



FIG. 3



FIG. 4

INVENTOR

H. C. L. DUNKER

BY *Wendroth, Lind & Poack*

ATTORNEYS

1

2,896,949

## TENNIS BALLS

Henry Christian Louis Dunker, Helsingborg, Sweden

Application March 15, 1954, Serial No. 416,258

Claims priority, application Sweden August 22, 1950

11 Claims. (Cl. 273—61)

This application is a continuation-in-part of applicant's co-pending application Serial No. 238,197, filed July 23, 1951, and Serial No. 266,443, filed January 24, 1952, both now abandoned.

The present invention relates to improvements in tennis balls.

Ordinary tennis balls generally consist of an inner hollow core of rubber (rubber ball) having a gas filling under super-atmospheric pressure and a covering of felt attached to the outside of said core. The structural characteristics of the ball, such as the composition of the rubber, the wall thickness and the diameter of the rubber core, the amount of super-atmospheric pressure, and the nature of the felt covering, may be varied within relatively narrow limits since these characteristics are required to impart predetermined properties to the ball with respect to the outer diameter, weight, hardness and rebound.

These requirements are defined in the "Rules of Lawn Tennis" as laid down by the International Tennis Federation. According to these specifications, a tennis ball shall be more than 2½ inches and less than 2½ inches in diameter, and not less than 2 ozs. (56.7 gr.) nor more than 2½ ozs. (58.5 gr.) in weight, and the ball shall have a minimum rebound of 53 inches (135 cm.) and a maximum rebound of 58 inches (147 cm.) when dropped 100 inches (254 cm.) and a deformation of not less than .265 of an inch and not more than .290 of an inch when subjected to a pressure of 18 lbs.

In a tennis ball which is made so as to comply with the requirements of diameter and weight, the proper hardness and rebound properties are generally attained by suitably adjusting the super-atmospheric pressure of the gas filling within the rubber core. However, the finished ball will not keep these properties unchanged for any considerable period of time, because the gas under pressure gradually diffuses out through the rubber wall, and thereby results in a reduction of both the hardness and the rebound of the ball.

Attempts have already been made to avoid these difficulties by varying the pressure of the gas filling and by increasing the impermeability of the rubber covering. For example, it has been proposed to stiffen the rubber core by means of a network of ribs on the interior surface thereof. However, none of the proposed solutions to the problem of storage has been successful in practice.

The principal object of the present invention is to provide an improved tennis ball in which the requirement of having a gas filling of super-atmospheric pressure is dispensed with and which, owing to the absence of a pressure differential between the inside and outside of the modified rubber core, will maintain its original proper hardness and rebound properties for a long period of time.

It is a further object of the invention to provide a tennis ball comprising a hollow modified rubber core having an outer diameter and a wall thickness similar to

2

those of tennis balls in general use but containing a gas filling at atmospheric pressure, while displaying the required hardness and rebound properties.

Another object of the invention is to provide a tennis ball comprising a hollow modified rubber core containing a gas filling at atmospheric pressure, and an outer felt covering, said ball being similar in appearance and playing properties to tennis balls which satisfy the International and National Tennis Association requirements but having substantially improved keeping qualities and, as a consequence thereof, a prolonged playing life.

A further object of the invention is to provide a tennis ball comprising a hollow modified rubber core containing a gas filling at atmospheric pressure, and an outer covering serving to give the ball the surface characteristics required in official match play, said tennis ball being capable of being stored for a prolonged time period without any falling-off in its hardness and rebound properties.

According to the present invention, the above and other objects are attained in a tennis ball, comprising a hollow rubber structure by having incorporated in said structure an ingredient consisting of a resinous high styrene-butadiene copolymer.

The accompanying drawing illustrates examples of tennis balls in accordance with the present invention. Figures 1 to 3, inclusive, show cross-sections of tennis balls in accordance with the invention.

In Figures 1-3, the tennis ball comprises a molded and cured rubber composition 4 containing rubber, rubber processing ingredients and a high styrene-butadiene copolymer, the ball being filled with a gas 2 at substantially atmospheric pressure. In Figs. 1 and 3 a covering of textile material 3 is shown. In Fig. 2 a covering of sponge rubber 3' is shown.

In Figs. 1 and 2, the tennis ball comprises a dual layered structure, the inner layer 1 being made from a molded and cured rubber composition of the well-known type and the outer layer 4 being composed of a composition of rubber, rubber processing ingredients, and a high styrene-butadiene copolymer. A surface layer or covering 3 of felt is applied to said rubber structure. Figure 4 illustrates a detail of a tennis ball in a modification of Fig. 3, the detail consisting of a dual layer rubber structure, in which the inner layer 7 is composed of an ordinary rubber composition and the outer layer 8 of a rubber composition including a high styrene-butadiene copolymer, said outer layer 8 being of a spongy character, so that no felt covering is needed.

Resinous copolymers of styrene and butadiene containing at least 50% by weight of styrene are known to stiffen rubber. It has been found that they increase the hardness and rigidity of the rubber stock. In general, they also improve the tensile strength, toughness, and resistance to tear and abrasion of rubber. Therefore, such copolymers have been found useful as stiffening and reinforcing agents in rubber soles and similar articles where the hardness and abrasion resistance of the rubber is of primary importance, *inter alia* in golf ball, soft ball and basket ball covers.

Applicant has found by incorporating such resinous high styrene-butadiene copolymers in the rubber structure of tennis balls that properly matched hardness and rebound characteristics of the finished balls may be produced in the absence of super-atmospheric gas pressure filling within the hollow rubber structure. On the basis of the knowledge of the influence of such copolymers on the properties of rubber stock, it was to be expected that an increased hardness of the rubber structure of tennis balls would result from the incorporation of the copolymers in the rubber. A similar increase in hardness is

observed upon adding such well-known ingredients to the rubber, as inorganic fillers such as kaolin or chalk. It was surprising to discover, that despite an increase in hardness the remaining resilience of the rubber stock is remarkably effective in tennis balls to permit the objectionable super-atmospheric pressure within the balls to be dispensed with. Particularly, in view of the reduction in the resilience of the rubber caused by the copolymer, it was not expected that tennis balls made from such rubber stock and having a gas filling of atmospheric pressure could possess the proper weight and hardness and also comply with the requisite rebound specification under the international rules.

One example of a resinous high styrene-butadiene copolymer which is suitable for the purposes of the present invention is a product sold by the B. F. Goodrich Chemical Company under the trade name of "Goodrite Resin 50" and consisting of about 85% styrene and 15% butadiene. This resin is described for example in an article "Rubber or Plastics" in the "Modern Plastics," July 1948. Other examples are a product sold by the Marbon Corporation under the name of "Marbon B" and a product sold by the Dewey and Almy Chemical Co. under the name of "Darex Copolymer 3," both consisting of 70% styrene and 30% butadiene. A further example is a product sold by the Polymer Corporation, Ltd., of Canada, under the same of SS-250, and consisting of 55% styrene and 45% butadiene. Still another example is a product sold by the Goodyear Tire & Rubber Company under the name of "Pliolite S-3." The important characteristics of this product are explained in an article "Styrene-Diene Resins in Rubber Compounding" by A. M. Borders et al. in the "Industrial and Engineering Chemistry," vol. 38—1946. Further examples of suitable copolymers are products sold by the Marbon Corporation and known under the names of "Marbon S and S1," which are described in an article "High Styrene Resins in Rubber Compounding" by A. G. Susie et al. in the "Rubber Age," August 1949.

A tennis ball embodying the present invention may consist of an inner hollow rubber body having uniformly incorporated therein by conventional rubber handling procedures a high styrene-butadiene copolymer and an outer covering of the usual felt material or a material having characteristics equivalent to those of such felt material, such as sponge rubber, the said body enclosing a gas filling, preferably air at ordinary atmospheric pressure. The rubber blend from which the said rubber body is made may, apart from ordinary fillers and processing ingredients such as kaolin, accelerators, and sulphur, preferably contain from about 65 to about 90 parts of rubber and from about 10 to about 35 parts of a high styrene-butadiene copolymer. Where a copolymer very high in styrene, e.g. containing about 85% styrene and about 15% butadiene ("Goodrite Resin 50"), is used, an amount of said copolymer at the lower part of said range is required, whereas a copolymer lower in styrene will as a rule be added to the rubber in amounts nearer the upper limit of said range, in order that the finished tennis balls shall have the desired hardness and rebound properties. However, the application is not restricted to the exact ranges of the constituents mentioned above, since these may be varied somewhat so that the proportions may sometimes be a little outside of these ranges.

It is to be understood that the amount of resinous high styrene-butadiene copolymer incorporated with the rubber is an amount sufficient to prevent the resilience of the finished ball from dropping below a minimum value which will reduce the rebound properties as are necessary to comply with the Lawn Tennis specification, and at the same time the amount is sufficient to render the core substantially impermeable so that it will have the compressibility, hardness, wall thickness and weight characteristics despite modification by conventional filler ingredients.

In a laminated core construction the copolymer rubber mix may be even higher in copolymer content in the inner core to produce a tennis ball meeting the Lawn Tennis specifications and having the same unexcelled storage

5 characteristics as the single layered core. Further, the single layered core modified at its surface with a blowing agent possesses such an excellent balance of properties within the specification requirements so that the usual felt covering may be entirely dispensed with.

10 The characteristics of the finished balls are only slightly influenced by varying other factors, such as the proportion of kaolin or other filler in the rubber blend and the processing operations, mastication, rate of curing, etc. The wall thickness of the rubber body, and the nature of

15 the outer covering are as required for the hardness and rebound specifications as are also the weight and diameter of the balls.

A typical example of a rubber-copolymer composition within the above-mentioned limits which may be used for

20 making tennis balls as described is as follows:

## EXAMPLE 1

|                                               | Parts by weight |
|-----------------------------------------------|-----------------|
| Rubber                                        | 100             |
| 25 Resinous copolymer (85% styrene, 15% buta- | 30              |
| diene)                                        |                 |
| Zinc oxide                                    | 5               |
| Kaolin                                        | 20              |
| Stearic acid                                  | 2               |
| 30 Accelerator                                | 1               |
| Sulphur                                       | 2.5             |

The rubber blend is processed as is usual in rubber manufacture, and the ball cores are made therefrom using any well-known forming and curing technique

35 except that the means for developing super-atmospheric pressure within the cores are dispensed with. The application of the outer covering of felt material or any other equivalent material is also carried out in the well-known manner.

40 It is within the purview of the invention to produce tennis balls in which the hollow rubber structure includes an inner hollow rubber core containing a gas filling of atmospheric pressure and a rubber layer surrounding said core and having the resinous high styrene-butadiene copolymer incorporated therein. Since the said rubber layer containing the copolymer is here relied upon to impart to the balls the necessary hardness and rebound properties, otherwise obtained by having the gas filling at super-atmospheric pressure, and since this layer constitutes only part of the thickness of the rubber structure as a whole, the range of percentages of the copolymer in the rubber of said layer will be moved upwardly to some extent. For example, in using a copolymer containing 85% styrene and 15% butadiene ("Goodrite Resin 50") at least 15% of this copolymer may have to be included in the rubber blend, and in using a copolymer containing 70% styrene and 30% butadiene ("Marbon B") the proportion of copolymer in the rubber blend may be increased towards 50%. Typical examples

45 of rubber-copolymer compositions which may be used for this variety of tennis balls are as follows (the figures

50 being parts by weight):

| 65 Example                | 2   | 3   | 4   |
|---------------------------|-----|-----|-----|
| Natural Rubber            | 80  | 70  | 50  |
| Synthetic Rubber ("GR-S") | 20  | 30  |     |
| "Marbon S"                |     |     | 50  |
| "Marbon S1"               |     |     | 50  |
| Zinc oxide                | 10  | 10  | 10  |
| 70 Stearic acid           | 2   | 2   | 2   |
| Mineral oil               |     |     | 5   |
| Accelerator               | 1.7 | 1.9 | 1.6 |
| Antioxidant               | 0.5 | 0.5 | 0.5 |
| Sulphur                   | 2.5 | 2.5 | 2.5 |

75 The rubber blends, after being processed, are prefer-

ably formed into sheets in a pressure curing operation carried out in a well-known manner. From these sheets are then stamped pieces of a desired shape which are coated with a cement and applied as a covering around the inner cured rubber core.

The hollow rubber structure, comprising the inner hollow rubber core and the outer covering of a rubber-copolymer composition, may have a surface layer of the usual felt material applied thereto. It is a further aspect of the invention that the said covering of a rubber-copolymer composition may be made spongy and, if desired, formed with any suitable surface pattern to make the said covering more or less equivalent to a felt layer and to provide a better grip to the ball and confine it to a smooth path through the air, thereby making an additional felt surface layer superfluous. The covering may be made spongy by adding to the rubber-copolymer compositions, for example those mentioned as Example Nos. 2, 3 and 4 above, so called blowing agents, e.g. ammonium carbonate, bicarbonate of soda, ammonium nitrate, azo compounds (sometimes used under the trade names of "Unicel," "Vulkacel," "Porofor," etc.) and others, in amounts of about 6 to 7 parts in the formulas of Examples 2, 3 and 4. Owing to the gases which these substances release on heating when the rubber is cured, the rubber becomes more or less spongy. The sponginess of the covering makes it lighter and reduces the rebound and hardness characteristics of the tennis balls, which has to be taken into account in designing the rubber structure. Thus, by varying the composition of the rubber-copolymer blend, particularly the ratio of rubber to copolymer and the amount of blowing agent, the rebound and hardness of the finished tennis balls may thereby be effectively controlled.

To illustrate the improvement achieved by the invention a number of rubber compositions and tennis balls made therefrom, filled at atmospheric pressure have been tested, and an account thereof is given below. In these tests the rubber blends of various compositions are mixed with various proportions of a high styrene-butadiene copolymer or other ingredients (cyclized rubber, coumarone resin, or kaolin), the hardness and resilience of the rubber made from such rubber-copolymer mixtures are determined, tennis balls are made from these rubber mixtures, and the compression (the inverse of hardness) and the rebound of the balls determined. The hardness of the rubber material is determined by means of the well-known Shore durometer "A," and the resilience is tested by means of a Schob pendulum in which the degree of resilience of the test piece is determined by the rebound of the pendulum after falling down onto said piece, the test value expressed in percent of the total fall of the pendulum.

Tennis ball cores were made from the rubber mixtures in the ordinary way. In some of the experiments, bare ball cores (without an outer felt covering) were tested in respect to the rebounding capacity and compression; in others both bare ball cores and finished (felt covered) balls were tested, as indicated below.

In conformity with the accepted requirements quoted above, the rebound of the balls was measured after allowing the balls to fall from a height of 254 cms., and the compression was determined by means of a "Major & Stevens" machine, in which the deformation of the balls by a predetermined load is measured in thousands of inches.

**I. Comparative tests of rubber mixed with various amounts of high styrene-butadiene copolymer or cyclized rubber**

High styrene-butadiene copolymer ("Goodrite Resin 50") and cyclized rubber, respectively, was mixed with a rubber blend of the following composition in parts by weight:

**6 FORMULA A**

|                       |     |
|-----------------------|-----|
| Natural rubber        | 100 |
| Zinc carbonate        | 6.5 |
| Kaolin                | 43  |
| 5 Stearine            | 1.3 |
| Mercaptobenzothiazole | 1.9 |
| Diphenylguanidine     | .9  |
| Sulphur               | 3.3 |

The rubber material and the bare ball cores were tested as explained above.

The results are given in the following Tables I and II.

TABLE I

| Rubber | Admixture | Rubber compound + styrene-butadiene copolymer |            | Rubber compound + Cyclized rubber |            |
|--------|-----------|-----------------------------------------------|------------|-----------------------------------|------------|
|        |           | Hardness                                      | Resilience | Hardness                          | Resilience |
| 100    | 0         | 59                                            | 60         | 59                                | 60         |
| 85     | 15        | 69                                            | 53         | 67                                | 52         |
| 70     | 30        | 82                                            | 40         | 81                                | 31         |

TABLE II

[Balls made from 85 parts rubber + 15 parts styrene-butadiene copolymer or cyclized rubber.]

|             | Copolymer | Cyclized rubber |
|-------------|-----------|-----------------|
| Rebound     | 170       | 150             |
| Compression | 290       | 305             |
| Weight, g.  | 45        | 45              |

The rubber blend contained a relatively high percentage of kaolin. The results indicated in Table I show that by substituting high styrene-butadiene for part of the rubber a rubber material having increased hardness but reduced resilience can be obtained. In comparison, cyclized rubber gives an almost equal increase in hardness but a greater reduction in resilience. From Table II it may be seen that a ball in which the rubber material contains 15% copolymer, calculated on the basis of rubber + copolymer, has properties which might make it suitable as a tennis ball, while a ball having part of the rubber replaced by cyclized rubber appears to be less suitable, because the rebound has dropped too much. (The bare ball cores, such as tested, ought to have slightly greater amounts of rebound and compression than required for the finished balls.)

**H. Investigation of the connection between hardness and resilience of rubber and rebound and compression of balls made therefrom**

The rubber blends used in these experiments differed slightly from those employed in the experiments reported under I.

A first series of runs were conducted with two different rubber blends mixed with high styrene-butadiene copolymer ("Goodrite Resin 50"). The formulas of these blends are given below, and the results are summarized in the corresponding Tables III and IV for various amounts of high styrene-butadiene copolymer.

FORMULA B

|                       |     |
|-----------------------|-----|
| Natural rubber        | 100 |
| Zinc carbonate        | 10  |
| Kaolin                | 10  |
| Stearine              | 1.5 |
| Rosin                 | .5  |
| Mineral oil           | .5  |
| Mercaptobenzothiazole | 1.6 |
| Diphenylguanidine     | .8  |
| 75 Sulphur            | 3.0 |

7  
FORMULA C

|                       |     |
|-----------------------|-----|
| Natural rubber        | 100 |
| Zinc carbonate        | 10  |
| Kaolin                | 25  |
| Stearine              | 1.5 |
| Rosin                 | .5  |
| Mineral oil           | .5  |
| Mercaptobenzothiazole | 1.6 |
| Diphenylguanidine     | 1.8 |
| Sulphur               | 3.0 |

TABLE III

| Rubber in<br>Formula B | Styrene-<br>butadiene<br>copolymer | Rubber+Styrene-<br>Butadiene Copolymer |            | Bare ball core  |         |
|------------------------|------------------------------------|----------------------------------------|------------|-----------------|---------|
|                        |                                    | Hardness                               | Resilience | Compre-<br>sion | Rebound |
| 100                    | 0                                  | 50                                     | 66         | ~700            | 180     |
| 90                     | 10                                 | 59                                     | 70         | 550             | 186     |
| 80                     | 20                                 | 65                                     | 68         | 471             | 175     |
| 72.5                   | 27.5                               | 78                                     | 54         | 172             | 155     |
| 65                     | 35                                 | 86                                     | 47         | 71              | 130     |

TABLE IV

| Rubber in<br>Formula C | Styrene-<br>butadiene<br>copolymer | Rubber+Styrene-<br>Butadiene Copolymer |            | Bare ball core  |         |
|------------------------|------------------------------------|----------------------------------------|------------|-----------------|---------|
|                        |                                    | Hardness                               | Resilience | Compre-<br>sion | Rebound |
| 100                    | 0                                  | 54                                     | 70         | 620             | 180     |
| 90                     | 10                                 | 62                                     | 70         | 505             | 184     |
| 80                     | 20                                 | 69                                     | 63         | 362             | 168     |
| 72.5                   | 27.5                               | 83                                     | 52         | 136             | 149     |
| 65                     | 35                                 | 87                                     | 43         | 61              | 124     |

It is seen from Tables III and IV above that the hardness of the rubber increases rapidly with an increased percentage of copolymer. The resilience of the rubber, on the other hand, instead of steadily falling off with an increasing percentage of copolymer, passes through a slight maximum at a content of about 10% copolymer,

which is clearly seen in Table III. The bare ball cores also display a maximum of rebound at a content of about 5 to 10% copolymer in the rubber, which confirms the fact that good resilience of the rubber is of importance for the rebound of the ball. With such low copolymer content, however, the compression of the ball is much too high. To produce a ball having the desired properties and not containing a gas filling at super-atmospheric pressure a rubber-copolymer mixture containing a higher proportion of the copolymer is used while taking into account that the rebound is reduced at the same time, and all the more as the amount of kaolin in the rubber blend is increased.

Other series of runs were carried out with additional rubber blends according to the following Formulas D, E, and F mixed with various proportions of kaolin, coumarone resin, or high styrene-butadiene copolymer ("Goodrite resin 50"), respectively. In these experiments the compression, the rebound, and the weight of the bare ball cores, on the one hand, and the finished (felt covered) balls, on the other hand, were examined. The results are found in the following Tables V, VI and VII.

## FORMULA D

|    |                                |     |
|----|--------------------------------|-----|
| 25 | Natural rubber                 | 100 |
|    | Zinc oxide                     | 8   |
|    | Magnesium carbonate            | 20  |
|    | Coumarone resin                | 3   |
|    | Stearine                       | 1.5 |
| 30 | Benzoic acid                   | 1   |
|    | Mercaptobenzothiazolebisulfide | 1.2 |
|    | Diphenylguanidine              | .5  |
|    | Sulphur                        | 3.6 |

## FORMULA E

|    |                                |     |
|----|--------------------------------|-----|
| 35 | Natural rubber                 | 100 |
|    | Zinc carbonate                 | 12  |
|    | Kaolin                         | 8   |
|    | Stearine                       | 1   |
| 40 | Mercaptobenzothiazoledisulfide | 1.5 |
|    | Diphenylguanidine              | .8  |
|    | Sulphur                        | 2.8 |

TABLE V

| Kaolin per 100<br>parts of rubber in<br>Formula D | Rubber+Kaolin              |                             | Bare ball core                              |                      |               | Finished ball                               |                      |               |
|---------------------------------------------------|----------------------------|-----------------------------|---------------------------------------------|----------------------|---------------|---------------------------------------------|----------------------|---------------|
|                                                   | Hard-<br>ness<br>(Shore °) | Resil-<br>ience,<br>Percent | Compre-<br>sion,<br>inches .10 <sup>3</sup> | Re-<br>bound,<br>cm. | Weight,<br>g. | Compre-<br>sion,<br>inches .10 <sup>3</sup> | Re-<br>bound,<br>cm. | Weight,<br>g. |
| 0                                                 | 54                         | 68                          | 636                                         | 164                  | 44.2          | 510                                         | 126                  | 57.0          |
| 20                                                | 59                         | 69                          | 613                                         | 156                  | 47.9          | 453                                         | 126                  | 61.3          |
| 50                                                | 66                         | 66                          | 433                                         | 158                  | 53.1          | 314                                         | 134                  | 65.9          |
| 70                                                | 70                         | 61                          | 340                                         | 165                  | 56.4          | 251                                         | 140                  | 69.6          |
| 85                                                | 73                         | 60                          | 320                                         | 164                  | 57.4          | 231                                         | 140                  | 70.6          |
| 100                                               | 73                         | 58                          | 262                                         | 160                  | 60.0          | 216                                         | 142                  | 73.0          |

TABLE VI

| Coumarone per 100<br>parts of rubber in<br>Formula D | Rubber+<br>Coumarone       |                             | Bare ball core                              |                      |               | Finished ball                               |                      |               |
|------------------------------------------------------|----------------------------|-----------------------------|---------------------------------------------|----------------------|---------------|---------------------------------------------|----------------------|---------------|
|                                                      | Hard-<br>ness<br>(Shore °) | Resil-<br>ience,<br>Percent | Compre-<br>sion,<br>inches .10 <sup>3</sup> | Re-<br>bound,<br>cm. | Weight,<br>g. | Compre-<br>sion,<br>inches .10 <sup>3</sup> | Re-<br>bound,<br>cm. | Weight,<br>g. |
| 0                                                    | 54                         | 68                          | 636                                         | 164                  | 44.2          | 510                                         | 126                  | 57.0          |
| 10                                                   | 53                         | 62                          | 680                                         | 158                  | 44.6          | 515                                         | 120                  | 58.2          |
| 20                                                   | 48                         | 52                          | 680                                         | 130                  | 44.5          | 563                                         | 115                  | 57.8          |
| 30                                                   | 46                         | 38                          | 680                                         | 112                  | 44.3          | 650                                         | 104                  | 57.6          |
| 50                                                   | 42                         | 24                          | 680                                         | 40                   | 44.4          | 700                                         | 30                   | 57.5          |

TABLE VII

| Copolymer per 100 parts of rubber in Formula E | Rubber+Copolymer   |                     | Bare ball core                    |              |            | Finished ball                     |              |            |
|------------------------------------------------|--------------------|---------------------|-----------------------------------|--------------|------------|-----------------------------------|--------------|------------|
|                                                | Hardness (Shore °) | Resilience, Percent | Compression, inches $\times 10^3$ | Rebound, cm. | Weight, g. | Compression, inches $\times 10^3$ | Rebound, cm. | Weight, g. |
| 0                                              | 54                 | 68                  | 636                               | 164          | 44.2       | 510                               | 126          | 57.0       |
| 17.6                                           | 61                 | 68                  | 539                               | 182          | 44.2       | 395                               | 140          | 57.5       |
| 29                                             | 70                 | 64                  | 378                               | 182          | 44.3       | 284                               | 144          | 57.9       |
| 43                                             | 81                 | 52                  | 163                               | 158          | 44.4       | 157                               | 138          | 57.8       |

As will appear from the above tables, the finished balls are slightly harder and have less rebound than the bare ball cores.

With a major proportion of kaolin incorporated in the rubber, balls may be manufactured which have quite acceptable rebound and hardness characteristics, as seen in Table V. However, the weight of the balls becomes too great. If the wall of the balls is made thinner to reduce the weight, the hardness is reduced and the rebound is also altered. With less kaolin the hardness as well as the rebound become too low. Thus it is not possible by incorporating kaolin in the rubber to arrive at a ball which has the proper hardness, rebound and weight characteristics, without using an internal super-atmospheric pressure in the ball.

Coumarone resin (Table VI) which has approximately the same specific gravity as rubber may be added in greater amounts without appreciably affecting the weight of the ball. However, it reduces the hardness and resilience of the rubber material and also causes a reduction of the rebound and hardness characteristics of the ball. Therefore, such resin, alone, is not suitable as a rubber modifier for the present invention.

The specific gravity of high styrene-butadiene copolymer also differs insignificantly from that of rubber. It increases the hardness of the rubber material considerably, and reduces the resilience thereof. It lowers the rebound slightly but not more than kaolin.

It can clearly be seen from Table VII, however, that the rebound of the balls has a certain maximum which lies at a higher proportion of the copolymer component than the slight maximum which can be found for the resilience of the rubber material.

As exemplified by Table VII, a certain amount of kaolin may advantageously be incorporated in the rubber material. Other well-known fillers may also be present. It should be noted, however, that such fillers are not necessary ingredients in the rubber, when high styrene-butadiene copolymers are added, but they are used as means for the purpose of slightly adjusting the properties of the rubber and the balls made therefrom.

From Table VII it may be seen that the properties of the bare ball cores and those of the felt covered balls do not vary quite in unison, with varying proportions of copolymer in the rubber. Thus, while a soft ball becomes considerably less compressible through the felt covering, a hard ball does not change very much in respect of compressibility by the application of the felt covering. Similarly the rate of decrease of the rebound, with increasing percentages of copolymer in the rubber, is diminished by the felt covering.

Some further specific examples of rubber-copolymer compositions suitable for making tennis balls, having a gas filling of atmospheric pressure only, according to the present invention will now be given.

| Example                   | 5     | 6     | 7     |
|---------------------------|-------|-------|-------|
| Natural rubber            | 100   | 100   | 100   |
| Copolymer (86% styrene)   | 12    | 30    | 63    |
| Zinc carbonate            | 10    | 10    | 10    |
| Kaolin                    | 30    | 15    | —     |
| Stearine                  | 1.5   | 1.5   | 1.5   |
| Mineral oil               | —     | —     | .5    |
| Rosin                     | .5    | .5    | .5    |
| Mercaptobenzothiazole     | 1.6   | 1.6   | 1.6   |
| Diphenylguanidine         | 1.0   | .8    | .8    |
| Sulphur                   | 3.0   | 3.0   | 3.0   |
| Rubber:Copolymer, approx. | 89:11 | 77:23 | 66:35 |

  

| Example                   | 8     | 9     | 10    |
|---------------------------|-------|-------|-------|
| Natural rubber            | 100   | 100   | 100   |
| Copolymer (70% styrene)   | 16    | 41    | 79    |
| Zinc carbonate            | 12    | 12    | 16    |
| Kaolin                    | 35    | 20    | —     |
| Stearine                  | 1.5   | 1.5   | 1.5   |
| Mineral oil               | —     | —     | .5    |
| Rosin                     | .5    | .5    | .5    |
| Mercaptobenzothiazole     | 1.6   | 1.8   | 1.8   |
| Diphenylguanidine         | 1.0   | 1.0   | 1.0   |
| Sulphur                   | 3.0   | 3.0   | 3.0   |
| Rubber:Copolymer, approx. | 86:14 | 70:30 | 56:44 |

When using the extreme rubber-copolymer compositions represented by the above Examples 5, 7, 8 and 10, considerable difficulties are experienced to have the compressibility, rebound and weight within the limits required for tennis balls. This is borne out by the figures in Tables III and IV, which refer to rubber-copolymer compositions similar to those listed above.

Where the rubber structure of the tennis balls is made from an inner rubber core (not containing copolymer) and an outer covering of rubber-copolymer composition, the proportion of copolymer will have to be slightly greater, as already pointed out, and for this reason, the compositions of Examples 5 and 8 will hardly be practicable in such case, while Examples 6, 7, 9 and 10 may perform satisfactorily. Where a copolymer containing 85% styrene is used, a practical upper limit for the proportion of the copolymer in the composition appears to be about 45%.

It is thought that the invention and its advantages will be understood from the foregoing description and it is apparent that various changes may be made in the form, construction and arrangement of the parts without departing from the spirit and scope of the invention or sacrificing its material advantages, the forms hereinbefore described and illustrated in the drawings being merely preferred embodiments thereof.

Having thus disclosed the invention what is claimed is:

1. A tennis ball, comprising a hollow structure of rubber, and a resinous high styrene-butadiene copolymer incorporated in at least a spherical annulus of said structure in a proportion of 10 to 45 parts thereof per 90 to 55 parts of rubber, calculated on the basis of 85% styrene in said copolymer, and a gas filling within said hollow structure at substantially atmospheric pressure,

2. A tennis ball, comprising a hollow structure at substantially atmospheric inner pressure having a diameter of  $2\frac{1}{2}$  to  $2\frac{5}{8}$  inches and a weight of 2 to  $2\frac{1}{16}$  ozs., at least a core portion of said structure being of rubber, and at least a spherical layer of said core portion having incorporated therein a resinous high styrene-butadiene copolymer in a proportion of 12 to 80 parts thereof, calculated on the basis of 85% styrene in said copolymer, per 100 parts of rubber to impart concurrently to said structure a deformation characteristic of 0.265 to 0.290 of an inch under a pressure of 18 lbs. and a rebound characteristic of 53 to 58 inches after a drop of 100 inches.

3. A tennis ball, comprising a hollow structure at substantially atmospheric inner pressure having a diameter of  $2\frac{1}{2}$  to  $2\frac{5}{8}$  inches and a weight of 2 to  $2\frac{1}{16}$  ozs., at least a core portion of said structure being of rubber, and at least a spherical layer of said core portion having incorporated therein 12 to 80 parts of a resinous high styrene-butadiene copolymer, calculated on the basis of 85% styrene in said copolymer, and 10 to 47 parts of inorganic filler material per 100 parts of rubber, to impart concurrently to said structure a deformation characteristic of 0.265 to 0.290 of an inch under a pressure of 18 lbs. and a rebound characteristic of 53 to 58 inches after a drop of 100 inches.

4. A tennis ball, comprising a hollow structure at substantially atmospheric inner pressure having a diameter of  $2\frac{1}{2}$  to  $2\frac{5}{8}$  inches and a weight of 2 to  $2\frac{1}{16}$  ozs., at least a core portion of said structure comprising rubber, 12 to 53 parts of a resinous high styrene-butadiene copolymer, calculated on the basis of 85% styrene in said copolymer, and 10 to 40 parts of inorganic filler material per 100 parts of rubber, to impart concurrently to said structure a deformation characteristic of 0.265 to 0.290 of an inch under a pressure of 18 lbs. and a rebound characteristic of 53 to 58 inches after a drop of 100 inches.

5. A tennis ball, comprising a hollow structure at substantially atmospheric inner pressure having a diameter of  $2\frac{1}{2}$  to  $2\frac{5}{8}$  inches and a weight of 2 to  $2\frac{1}{16}$  ozs., at least a core portion of said structure comprising rubber, the outer spherical layer of said core portion having incorporated therein 30 to 53 parts of a resinous high styrene-butadiene copolymer, calculated on the basis of 85% styrene in said copolymer, and 10 to 25 parts of inorganic filler material per 100 parts of rubber, to impart concurrently to said structure a deformation characteristic of 0.265 to 0.290 of an inch under a pressure of 18 lbs. and a rebound characteristic of 53 to 58 inches after a drop of 100 inches.

6. A tennis ball, comprising a hollow structure at substantially atmospheric inner pressure having a diameter of  $2\frac{1}{2}$  to  $2\frac{5}{8}$  inches and a weight of 2 to  $2\frac{1}{16}$  ozs., at least a core portion of said structure comprising rubber, 16 to 79 parts of a resinous high styrene-butadiene copolymer, calculated on the basis of 70% styrene in said copolymer, and 15 to 47 parts of inorganic filler material per 100 parts of rubber, to impart concurrently to said structure a deformation characteristic of 0.265 to 0.290 of an inch under a pressure of 18 lbs. and a rebound characteristic of 53 to 58 inches after a drop of 100 inches.

7. A tennis ball, comprising a hollow structure at substantially atmospheric inner pressure having a diameter of  $2\frac{1}{2}$  to  $2\frac{5}{8}$  inches and a weight of 2 to  $2\frac{1}{16}$  ozs., at least a core portion of said structure being of rubber, the rubber in a spherical layer of said core portion having incorporated therein 41 to 79 parts of a resinous high styrene-butadiene copolymer, calculated on the basis of 70% styrene in said copolymer, and 15 to 32 parts of

inorganic filler material per 100 parts of rubber, to impart concurrently to said structure a deformation characteristic of 0.265 to 0.290 of an inch under a pressure of 18 lbs. and a rebound characteristic of 53 to 58 inches after a drop of 100 inches.

8. A tennis ball, comprising a hollow structure of rubber, a resinous high styrene-butadiene copolymer incorporated in at least a spherical layer of said structure in a proportion of 10 to 45 parts thereof per 90 to 55 parts of rubber, calculated on the basis of 85% styrene in said copolymer, a surface layer of a material having surface characteristics equivalent to those of felt material, and a gas filling within said hollow structure at substantially atmospheric pressure.

15 9. A tennis ball, comprising a hollow structure at substantially atmospheric inner pressure having a diameter of  $2\frac{1}{2}$  to  $2\frac{5}{8}$  inches and a weight of 2 to  $2\frac{1}{16}$  ozs., at least a core portion of said structure being of rubber, the rubber in at least a spherical layer of said core portion having incorporated therein a resinous high styrene-butadiene copolymer in a proportion of 12 to 80 parts thereof, calculated on the basis of 85% styrene in said copolymer, per 100 parts of rubber, to impart concurrently to said structure a deformation characteristic of 0.265 to 0.290 of an inch under a pressure of 18 lbs. and a rebound characteristic of 53 to 58 inches after a drop of 100 inches, and a surface layer of a material having surface characteristics equivalent to those of felt material.

20 10. A tennis ball, comprising a hollow structure at substantially atmospheric inner pressure having a diameter of  $2\frac{1}{2}$  to  $2\frac{5}{8}$  inches and a weight of 2 to  $2\frac{1}{16}$  ozs., at least a core portion of said structure being of rubber, the rubber in a spherical outer layer of said core portion having incorporated therein 30 to 53 parts of a resinous high 25 styrene-butadiene copolymer, calculated on the basis of 85% styrene in said copolymer, and 10 to 25 parts of inorganic filler material per 100 parts of rubber, to impart concurrently to said structure a deformation characteristic of 0.265 to 0.290 of an inch under a pressure of 18 lbs. and a rebound characteristic of 53 to 58 inches after a drop of 100 inches, and a surface layer of material having surface characteristics equivalent to those of felt material.

30 11. A tennis ball, comprising a hollow structure at substantially atmospheric inner pressure having a diameter of  $2\frac{1}{2}$  to  $2\frac{5}{8}$  inches and a weight of 2 to  $2\frac{1}{16}$  ozs., said structure having a spherical inner layer of rubber and a spherical outer layer of spongy rubber, the rubber of 35 which the spongy rubber is formed having incorporated therein 30 to 53 parts of a resinous high styrene-butadiene copolymer, calculated on the basis of 85% styrene in said copolymer, and 10 to 25 parts of inorganic filler material per 100 parts of rubber to impart concurrently to said 40 structure a deformation characteristic of 0.265 to 0.290 of an inch under a pressure of 18 lbs. and a rebound characteristic of 53 to 58 inches after a drop of 100 inches, and a surface layer of material having surface characteristics equivalent to those of felt material.

45 12. A tennis ball, comprising a hollow structure at substantially atmospheric inner pressure having a diameter of  $2\frac{1}{2}$  to  $2\frac{5}{8}$  inches and a weight of 2 to  $2\frac{1}{16}$  ozs., said structure having a spherical inner layer of rubber and a spherical outer layer of spongy rubber, the rubber of 50 which the spongy rubber is formed having incorporated therein 30 to 53 parts of a resinous high styrene-butadiene copolymer, calculated on the basis of 85% styrene in said copolymer, and 10 to 25 parts of inorganic filler material per 100 parts of rubber to impart concurrently to said 55 structure a deformation characteristic of 0.265 to 0.290 of an inch under a pressure of 18 lbs. and a rebound characteristic of 53 to 58 inches after a drop of 100 inches.

#### References Cited in the file of this patent

#### UNITED STATES PATENTS

|           |             |               |
|-----------|-------------|---------------|
| 1,402,682 | Takashima   | Jan. 3, 1922  |
| 1,614,853 | Schwartz    | Jan. 18, 1927 |
| 2,131,756 | Roberts     | Oct. 4, 1938  |
| 2,452,999 | Daly et al. | Nov. 2, 1948  |

#### OTHER REFERENCES

Industrial and Engineering Chemistry, September 1946, pp. 955-957.

India Rubber World, January 1948, pp. 487-491.

Modern Plastics, February 1950, pp. 72-74.